

April 12, 1949.

L. L. McMURRAY  
STARCH-CAUSTIC IN APATITE-ILMENITE  
FROTH FLOTATION  
Filed Dec. 20, 1945

2,466,995



## UNITED STATES PATENT OFFICE

2,466,995

STARCH-CAUSTIC IN APATITE-ILMENITE  
FROTH FLOTATIONLynn L. McMurray, Asheville, N. C., assignor to  
American Cyanamid Company, New York, N. Y.,  
a corporation of Maine

Application December 20, 1945, Serial No. 636,227

10 Claims. (Cl. 209—167)

1

This invention relates to the beneficiation by froth flotation of those metallic oxide ores containing excessive amounts of phosphate minerals. More particularly, it is concerned with the separation of phosphorous-bearing minerals such as apatite from metallic oxide minerals such as ilmenite, rutile, magnetite, hematite and the like.

The typical problems involved as well as their solutions are found in the production of ilmenite concentrates. In commercial practice, the use of titanium oxides has become increasingly important and accordingly the demand for high grade ore from which they may be recovered has steadily increased. Unfortunately, while there are many natural deposits of titanium minerals, the grade of these ores in many cases is not sufficiently high to make recovery of titanium oxides therefrom commercially feasible. Particularly is this true of most deposits within the United States. Therefore, while the process is not limited thereto, the invention will be illustrated by its application to titanium ores and ilmenite in particular.

Natural deposits of titanium-bearing minerals are usually ores containing, in addition to the titanium-bearing mineral such as ilmenite, rutile or the like, a silica-bearing gangue. Ordinarily, this silica and/or silicate content must be reduced to produce a concentrate meeting commercial standards, for example, to be used as raw material for the production of titanium oxide pigments.

Moreover, a problem with which the present invention is particularly concerned is presented by the fact that in addition to the silica or silicates, many ores, particularly in the United States, contain a certain amount of phosphorous-bearing minerals. In the illustrative case of ilmenite, this is frequently apatite. The presence of phosphorus is objectionable in a raw material for the production of titanium oxide pigments in their various crystal forms such as rutile or anatase. Particularly is this true in the latter case. A commercially acceptable concentrate must have a low  $P_2O_5$  content. Since the  $P_2O_5$  assay may vary from about 1-2% in ilmenite concentrates obtained from ores which are worked primarily for other constituents to 12% or more, as found in ilmenite ores such as nelsonite, the reduction of the  $P_2O_5$  content is essential. Those

processes which in the past have been employed to reduce the silica or silicate content are not effective for this purpose.

Despite the demand therefor, there has been available no process for readily and effectively producing concentrates of metallic oxides such as ilmenite or the like, sufficiently low in  $P_2O_5$  content. Neither have the concentrates previously obtainable always been in a satisfactory physical condition in which they can be readily dewatered and dried for further processing.

It is, therefore, a principal object of the present invention to provide a process by which a concentrate satisfactorily low in  $SiO_2$  and  $P_2O_5$  content can be obtained. It is also an object to provide a process whereby this is accomplished in an economical manner and with good recovery. It is a further object to provide suitable reagents for use in this process, which reagents are simple in use, readily obtainable and effective in operation.

It is with the reduction in the  $P_2O_5$  assay that the present invention is primarily concerned. Its practice, however, also effectively reduces the  $SiO_2$  assay in the final metallic oxide concentrate. In accordance with the present invention separation of apatite, for example, from a metallic oxide such as ilmenite, is made by preparing a deslimed feed, conditioning it with a novel depressant for the ilmenite and siliceous content, floating off the bulk of the apatite, repeating the flotation if the  $P_2O_5$  is not sufficiently reduced, removing any residual depressant, and taking the ilmenite concentrate from the residual solids by means of a similar type of promoter used for the apatite.

The invention will be discussed in conjunction with the accompanying drawing which delineates a typical flow scheme of a process involving the practice of the present invention.

In discussing flow scheme, and details of the present invention elsewhere throughout the specification, the separation of apatite

45  $Ca_5(Cl,F)(PO_4)_3$ 

a commonly-occurring phosphate, from ilmenite  $FeO \cdot TiO_2$  a typical metallic oxide, is described. However, the present invention is not to be construed as being limited to the separation of the

two latter mentioned minerals, but covers broadly the separation of phosphorous-bearing minerals from metallic oxides.

It is highly desirable that the selective apatite float be carried out with anionic-type reagents, if possible, since the latter not only are both simpler and more economical in use but produce a concentrate that can be more readily dewatered. Unfortunately apatite and most metallic oxide minerals, including ilmenite, react very much the same to most anionic type promoters. It is necessary therefore that a depressant be found for one constituent or the other. In accordance with the present invention depression of ilmenite is effectively accomplished with a novel group of agents. The feed is suitably conditioned with caustic selected from the group consisting of sodium, potassium and ammonium hydroxides, starch, and preferably also during the same conditioning operation, with an anionic-type promoter for the apatite.

Referring to the flow sheet it will be seen that the initial operations are concerned with preparing the ore. As shown in the drawing, this comprises grinding or otherwise reducing the ore to a suitable size for flotation, and removing the slimes. Any combination of crushing, grinding, and desliming steps may be used. In the case of many ores, it has been found to be good practice to crush the whole ore to about minus 10 mesh and then remove the primary slimes. This permits discarding a substantial portion of the original weight, usually with a very small loss of ilmenite. It is the deslimed material which forms the feed to the grinding circuit shown in the accompanying flow sheet. As shown, the feed is usually ground to less than minus 35 mesh and preferably to minus 50 or minus 60 mesh. Grinding is followed by a secondary desliming operation producing a deslimed product in suitable condition for further processing.

The deslimed sands are conditioned with the ilmenite depressants and the apatite promoter. This conditioning step is carried out at high solids although it may be done at flotation density if so desired. The ilmenite depressant may be referred to as caustic starch although the designation is a slight misnomer. The reagent actually comprises a mixture of an alkali such as sodium hydroxide and starch. Preferably it is fed as a solution containing about 5-10% dissolved solids. The alkali-starch ratio may vary from as little as about 5-1 to as high as about 30-1. It has been found that good results are obtained for most purposes using about 20 parts of caustic per part of starch. A sufficient amount should be used to produce depression of the ilmenite and to produce a pH of at least about 8.0-8.5 at flotation density, the solution being added and conditioned with the pulp for sufficient time to insure thorough dissemination.

At the same time the anionic promoter for the apatite is added. It has been found that this may be substantially any good anionic promoter of the fatty-acid or soap type. Good results are obtained with fatty acids such as oleic acid, fish-oil fatty acids, cocoanut-oil fatty acids and the like; with resin or naphthenic acids, talloel and the like. These may be used per se or as sodium, potassium or ammonium soaps thereof. Sulfonated reagents such as sulfonated or sulfated higher aliphatic alcohols; sulfonated fatty acids and fatty-acid-glyceride oils; sulfonated petroleum hydrocarbons of the "mahogany" and "green" types and the like may also be used

per se or as alkali-neutralized products but the strongly basic circuit does not permit their employment to best advantage.

Talloel has been found to give excellent results and since it is readily-available and relatively-inexpensive it is perhaps preferable. In general, the amount required is relatively small, from 0.25 to about 1.0 lb./ton of talloel per ton of flotation feed, or equivalent amounts of other reagents, being adequate for the majority of operations. In some few cases more may be required. Excessive amounts over that necessary to concentrate the apatite should be avoided as tending to overcome the effect of the ilmenite depressant. It appears to make little difference whether the talloel is added per se or in a pre-saponified form since there is enough alkali present to assure saponification in situ during conditioning.

After conditioning, the pulp is subjected to flotation. If conditioning was at high solids the pulp is first reduced to flotation density of from 15-20% solids. Flotation is carried out until the apatite removal is apparently complete. This initial flotation operation will be found to float and concentrate the major portion of the apatite content in the feed. In some cases, the apatite removal is sufficiently complete. The residual apatite content of the initial flotation tailing may be too high to meet specifications for a good ilmenite concentrate. Therefore, as shown in the drawing, the conditioning and flotation procedures are usually advantageously repeated taking off a second apatite concentrate or middling product and leaving a tailing of satisfactorily low  $P_2O_5$  content.

These apatite concentrates may be treated in any suitable manner. As shown in the drawing, the apatite concentrates are combined and subjected to a cleaner and recleaner flotation, the tailings from which are recycled to the grinding step but may be discarded if so desired. The resultant product is a clean, saleable, apatite concentrate.

To obtain the final ilmenite concentrate, the machine discharge or tailing, from the apatite concentrating is treated to remove any residual depressant, conditioned with an ilmenite promoter and a pulp-conditioning agent. As shown in the drawing, the residual depressant may be simply washed out of the apatite tailings before further treatment of the latter. However, as shown, it is preferable that the tailings be given an acid washing before the ilmenite flotation. The pulp-conditioning agent may be either an alkali or an acid. When an alkali is used it is added in a sufficient amount to produce a pH of at least about 8.0-8.5. The alkali usually employed is caustic soda, but if the occasion warrants, it may be substituted by potassium or ammonium hydroxide. The use of caustic alkali is probably the most conventional, because of its greater availability and lower cost.

In using acid as the pulp-conditioner it has been found that it is possible in some cases to reduce the  $SiO_2$  assay of the ilmenite concentrate somewhat. The inorganic acid usually used is sulfuric acid. However, an organic acid such as acetic acid also has been successfully used. From this it is apparent that the nature of the acid is not critical. Where the ilmenite concentration is being carried out in conjunction with the manufacture of titanium pigments, so-called "end liquor," comprising about 20% sulfuric acid

and 10%  $\text{FeSO}_4$  is usually available. This may be used. The amounts required are small as compared with the usual amount of alkali used, being generally in the neighborhood of 0.1-0.5 lb. of  $\text{H}_2\text{SO}_4$  or the equivalent, per ton of feed. The amount used in this way is small enough so that its effect is probably one of activating the ilmenite somewhat rather than a scrubbing or cleaning. The promoter used may be the same or a different anionic reagent from that used in concentrating apatite. Again talloel is perhaps the preferred reagent. It is generally added per se since pre-saponification would be useless in the presence of acid although it will occur in situ when alkali is used.

As shown in the drawing, the acid treatment is preferably carried out as a separate step. From about 5 to 10 lbs. of acid per ton of feed is usually found adequate. After thoroughly agitating the pulp-acid mixture, it is dewatered and washed thoroughly. Two or three washings are used to remove substantially all the excess acid. This washed pulp is then used as feed in the ilmenite flotation. In using this special acid washing step it is possible to leave a trace of acid in the pulp and simply condition with it the promoter for the ilmenite thus simply providing an acid source if the ilmenite flotation is to be done in acid circuit. On the other hand, it is perhaps preferable to use an alkaline circuit for the ilmenite flotation. The acid is washed out quite completely.

As shown in the drawing, whether the acid or alkali treatment is used, the pulp which has been reconditioned is fed to the ilmenite flotation circuit and an ilmenite concentrate removed. This rougher concentrate is usually given one cleaning by reflootation, and preferably at least another additional cleaning. The tailings from the ilmenite cleaner and recleaner flotation operations may be discarded if so desired. Usually at least the recleaner tailing may be advantageously recycled to the grinding operation.

The invention will be further illustrated in conjunction with the following examples which are intended as illustrative only. All parts are by weight unless otherwise noted. The ore treated in the following examples was a Nelsonite ore containing in addition to ilmenite, rutile, magnetite, and hematite, apatite and siliceous gangue minerals. Before the treatment shown in the following examples the ore had been reduced to minus 10 mesh and hydraulically deslimed.

#### EXAMPLE 1

In order to show the effectiveness of the starch-caustic as an ilmenite depressant, a sample of the ore was ground to minus 65 mesh and deslimed, the slimes being discarded. Sands as a thick pulp were conditioned for 1½ minutes with the reagents designated "group I" in Table I and an apatite concentrate (No. 1) floated for 6 minutes. This first apatite concentrate was cleaned once, the cleaner tailing being designated "Midd" in Table I. The tailings from this initial flotation operation were dewatered to a thick pulp and conditioned again for 1½ minutes with the reagents designated "group II" and a second apatite concentrate (No. 2) was floated. The tailings from the second apatite flotation were washed and dewatered, conditioned for 1½ minutes with the reagents designated "group III" and an ilmenite rougher concentrate removed for about 6 minutes. The ilmenite rougher concentrate was cleaned three times, the various cleaner

tailings being combined and designated "ilmenite middlings" as shown in Table I.

The reagents used and the metallurgical results are shown in the following Table I.

Table I

|    | Product             | Percent Weight | Assay                  |                | Recovery               |                |
|----|---------------------|----------------|------------------------|----------------|------------------------|----------------|
|    |                     |                | $\text{P}_2\text{O}_5$ | $\text{TiO}_2$ | $\text{P}_2\text{O}_5$ | $\text{TiO}_2$ |
| 10 | Caustic.....        |                | 6.0                    |                | 6.0                    |                |
|    | Starch.....         |                | 1.0                    |                | 1.0                    |                |
|    | Talloel.....        |                | 2.59                   |                | 2.59                   |                |
|    |                     |                |                        |                |                        | 1.08           |
| 15 |                     |                |                        |                |                        |                |
| 20 | Apattite No. 1..... | 20.7           | 34.0                   | 5.4            | 83.5                   | 3.9            |
|    | Apattite No. 2..... | 4.0            | 4.4                    | 15.0           | 2.1                    | 2.1            |
|    | Midds.....          | 6.3            | 14.9                   | 16.0           | 11.1                   | 3.5            |
|    | Ilm. Conc.....      | 40.2           | 0.11                   | 45.9           | 0.5                    | 64.3           |
|    | Ilm. Midds.....     | 22.8           | 0.99                   | 28.2           | 2.7                    | 22.4           |
|    | Final Tailing.....  | 6.0            | 0.74                   | 18.1           | 0.1                    | 3.8            |
| 25 | Feed (Calc.).....   | 100.0          | 5.50                   | 31.3           | 100.0                  | 100.0          |

#### EXAMPLE 2

Another sample of the ore was treated in the same way as in Example 1, except that the two apatite concentrates were combined and cleaned twice to produce a final apatite concentrate, the cleaner tailings being combined and designated "apatite Midds 1 and 2" in Table II. Also, the ilmenite rougher concentrate was cleaned only twice, the combined cleaner tailings being designated "ilmenite Midds 1 and 2" as shown in Table II. The reagents and results are shown in the following Table II.

Table II

|    | Product                           | Per cent Weight | Analysis per cent      |                | Recovery per cent      |                |
|----|-----------------------------------|-----------------|------------------------|----------------|------------------------|----------------|
|    |                                   |                 | $\text{P}_2\text{O}_5$ | $\text{TiO}_2$ | $\text{P}_2\text{O}_5$ | $\text{TiO}_2$ |
| 45 | Caustic.....                      |                 | 6.0                    |                | 3.0                    |                |
|    | Starch.....                       |                 | 0.5                    |                | 0.2                    |                |
|    | Talloel.....                      |                 | 1.6                    |                | 0.8                    |                |
|    | PH.....                           |                 |                        |                |                        | 8              |
| 50 |                                   |                 |                        |                |                        |                |
| 55 |                                   |                 |                        |                |                        |                |
| 60 | Apattite Conc.....                | 16.8            | 38.3                   | 2.1            | 85.5                   | 1.2            |
|    | Apattite Midds. 1 and 2.....      | 11.5            | 7.6                    | 12.5           | 11.4                   | 4.8            |
|    | Ilmenite Conc. <sup>1</sup> ..... | 57.9            | 0.2                    | 44.8           | 1.3                    | 87.3           |
|    | Ilmenite Midds. 1 and 2.....      | 8.2             | 1.1                    | 20.2           | 1.2                    | 5.6            |
|    | Final Tailing.....                | 5.6             | 0.9                    | 6.1            | 0.6                    | 1.1            |
| 65 | Feed (Calc.).....                 | 100.0           | 7.5                    | 29.7           | 100.0                  | 100.0          |

<sup>1</sup>  $\text{SiO}_2$ —1.24%; analysis.

#### EXAMPLE 3

In order to illustrate the beneficial effect of an acid wash in reducing the silica content of the ilmenite concentrate, Example 2 was repeated exactly except that the ilmenite flotation feed was conditioned for 5 minutes with 10 lbs./ton of 93%  $\text{H}_2\text{SO}_4$  and the sands were washed twice. To overcome any residual acid, the caustic content of the reagent group 3 was raised to 1.0 lb./ton. The results are shown in the following Table III.

Table III

| Product                     | Per cent Weight | Analysis per cent             |                  | Recovery per cent             |                  |
|-----------------------------|-----------------|-------------------------------|------------------|-------------------------------|------------------|
|                             |                 | P <sub>2</sub> O <sub>5</sub> | TiO <sub>2</sub> | P <sub>2</sub> O <sub>5</sub> | TiO <sub>2</sub> |
| Apatite Conc.               | 12.5            | 39.4                          | 1.1              | 88.8                          | 0.4              |
| Apatite Midds. 1 and 2      | 6.1             | 5.2                           | 24.5             | 5.8                           | 4.8              |
| Ilmenite Conc. <sup>1</sup> | 56.5            | 0.1                           | 46.7             | 1.1                           | 81.3             |
| Ilmenite Midds. 1, 2, 3     | 8.5             | 0.7                           | 37.4             | 1.1                           | 10.2             |
| Silicate Gangue             | 16.4            | 1.1                           | 6.3              | 3.2                           | 3.3              |
| Feed (Calc.)                | 100.0           | 5.5                           | 31.2             | 100.0                         | 100.0            |

<sup>1</sup> SiO<sub>2</sub>—0.62% ; analysis.

EXAMPLE 4

In order to illustrate the effect of carrying out the ilmenite flotation in the presence of acid, Example 2 was repeated except that in reagent group 3 sulfuric acid (98%) was used instead of caustic. The reagent quantities and illustrative results are shown in the following Table IV.

Table IV

| Product                        | Per cent Weight | Analysis per cent             |                  | Recovery per cent             |                  |
|--------------------------------|-----------------|-------------------------------|------------------|-------------------------------|------------------|
|                                |                 | P <sub>2</sub> O <sub>5</sub> | TiO <sub>2</sub> | P <sub>2</sub> O <sub>5</sub> | TiO <sub>2</sub> |
| Caustic                        |                 | 6.0                           |                  | 6.0                           |                  |
| Starch                         |                 | 0.5                           |                  | 0.5                           |                  |
| Talloel                        |                 | 1.6                           |                  | 1.6                           |                  |
| H <sub>2</sub> SO <sub>4</sub> |                 |                               |                  | 1.2                           | 0.2              |
|                                |                 |                               |                  |                               |                  |
| Apatite Conc.                  | 14.9            | 38.2                          | 1.9              | 85.9                          | 0.9              |
| Apatite Midds. 1 and 2         | 11.3            | 6.0                           | 20.3             | 10.2                          | 7.6              |
| Ilmenite Conc. <sup>1</sup>    | 51.0            | 0.14                          | 45.8             | 1.1                           | 77.6             |
| Ilmenite Midds. 1 and 2        | 17.1            | 0.8                           | 26.4             | 2.1                           | 13.1             |
| Silicate Gangue                | 5.7             | 0.8                           | 4.0              | 0.7                           | 0.8              |
| Feed (Calc.)                   | 100.0           | 6.6                           | 29.9             | 100.0                         | 100.0            |

<sup>1</sup> SiO<sub>2</sub>—0.84% ; analysis.

I claim:

1. A method of separating phosphorous-bearing minerals from mixtures thereof containing at least one metallic oxide mineral which comprises the steps of subjecting an aqueous pulp of the mixture to froth flotation in the presence of starch and a member of the group consisting of the sodium, potassium and ammonium hydroxides the starch-alkali ratio ranging from 1:5 up to 1:30 and a sufficient amount being used to produce a pH of at least 8 and to effectively depress substantially all of the metallic oxide mineral content and a sufficient amount of an anionic-type promoter selected from the long-chain fatty acid, resin acid, naphthenic acid types, talloel, their soluble soaps and mixtures thereof to float selectively the major portion of the phosphorous-bearing minerals.

2. A method of separating apatite from mixtures thereof containing at least one metallic oxide mineral which comprises the steps of subjecting an aqueous pulp of the mixture to froth flotation in the presence of starch and a member of the group consisting of the sodium, potassium and ammonium hydroxides the starch-alkali ratio ranging from 1:5 up to 1:30 and a sufficient amount being used to produce a pH of at least 8 and to effectively depress substantially all of the metallic oxide mineral content and a sufficient amount of an anionic-type promoter selected from the long-chain fatty acid, resin acid, naph-

thenic acid types, talloel, their soluble soaps and mixtures thereof to float selectively the major portion of the apatite.

3. A method of separating phosphorous-bearing minerals from mixtures thereof containing at least one titanium-bearing oxide mineral which comprises the steps of subjecting an aqueous pulp of the mixture to froth flotation in the presence of starch and a member of the group consisting of the sodium, potassium and ammonium hydroxides the starch-alkali ratio ranging from 1:5 up to 1:30 and a sufficient amount being used to produce a pH of at least 8 and to effectively depress substantially all of the titanium-bearing oxide mineral content and a sufficient amount of an anionic-type promoter selected from the long-chain fatty acid, resin acid, naphthenic acid types, talloel, their soluble soaps and mixtures thereof to float selectively the major portion of the phosphorous-bearing minerals.

4. A method of separating apatite from mixtures thereof containing at least one titanium-bearing oxide mineral which comprises the steps of subjecting an aqueous pulp of the mixture to froth flotation in the presence of starch and a member of the group consisting of the sodium, potassium and ammonium hydroxides the starch-alkali ratio ranging from 1:5 up to 1:30 and a sufficient amount being used to produce a pH of at least 8 and to effectively depress substantially all of the titanium-bearing oxide mineral content and a sufficient amount of an anionic-type promoter selected from the long-chain fatty acid, resin acid, naphthenic acid types, talloel, their soluble soaps and mixtures thereof to float selectively the major portion of the apatite.

5. A process according to claim 1 in which the alkali and starch are fed as an aqueous fluid solution thereof, this solution being added to the aqueous pulp and agitated therewith before the pulp is subjected to froth flotation.

6. A method of separating phosphorous-bearing minerals from mixtures thereof containing at least one metallic oxide mineral which comprises the steps of subjecting an aqueous pulp of the mixture to froth flotation in the presence of starch and a member of the group consisting of the sodium, potassium and ammonium hydroxides the starch-alkali ratio ranging from 1:5 up to 1:30 and a sufficient amount being used to produce a pH of at least 8 and to effectively depress substantially all of the metallic oxide mineral content and a sufficient amount of an anionic-type promoter selected from the long-chain fatty acid, resin acid, naphthenic acid types, talloel, their soluble soaps and mixtures thereof to float selectively the major portion of the phosphorous-bearing minerals, subjecting the tailing therefrom to a second froth flotation operation with the same reagent combination, whereby substantially all the residual phosphorous-bearing minerals are removed therefrom.

7. A method of separating apatite from mixtures thereof with titanium-bearing oxide minerals and silica-bearing gangue, which comprises the steps of making an aqueous pulp of the mixture; removing substantially all of the apatite from the pulp, by conditioning the pulp with causticized starch and an anionic-type promoter for the apatite, selected from the long-chain fatty acid, resin acid, naphthenic acid types, talloel, their soluble soaps and mixtures thereof, subjecting the conditioned pulp to froth flotation, collecting the froth concentrate which floats and removing the collected froth concentrate from

the circuit; washing the residual causticized starch from the residual solids; conditioning the latter with an anionic-type promoter for the titanium-bearing oxide mineral, selected from the noted promoters for apatite, and subjecting the 5 pulp to froth flotation, whereby a titanium-bearing concentrate having a silica assay low enough to be commercially acceptable is obtained.

8. A process according to claim 7 in which the titanium-bearing oxide mineral flotation is carried out in the presence of a small amount of free strong acid.

9. A process according to claim 7 in which the titanium-bearing oxide mineral flotation is carried out in the presence of sufficient alkali to 15 produce an alkaline pH.

10. A process according to claim 7 in which the residual solids from the apatite flotation are agitated with a small amount of a free strong acid and then washed substantially free therefrom before being conditioned with the titanium-bearing oxide mineral promoter.

LYNN L. McMURRAY.

#### REFERENCES CITED

10 The following references are of record in the file of this patent:

#### UNITED STATES PATENTS

| Number    | Name     | Date          |
|-----------|----------|---------------|
| 1,914,695 | Lange    | June 20, 1933 |
| 2,288,497 | Tartaron | June 20, 1942 |